

## UNITED STATES PATENT OFFICE.

REED P. ROSE, OF JACKSON HEIGHTS, AND HAROLD E. CUDE, OF FLORAL PARK, NEW YORK, ASSIGNORS TO GENERAL RUBBER COMPANY, OF NEW YORK, N. Y., A CORPORATION OF NEW JERSEY.

## SATURATING PAPER.

No Drawing.

Application filed December 11, 1925. Serial No. 74,889.

The present invention is concerned with the manufacture of a paper which has the capacity of absorbing aqueous emulsions of rubber, glue-glycerine combinations and other saturating compositions.

Saturating papers as heretofore made comprise in general blotting papers, gasket and similar materials and waterproof papers made by saturating methods. Blotting papers are ordinarily made from cotton fibre which is given a severe chemical treatment to remove fats, oils, waxes, and ligneous substance, and to disintegrate the cotton fibre itself. Fairly high concentrations of caustic soda and comparatively long cooking periods and high temperatures are employed to accomplish this purpose. Or the time may be shortened by elevating the temperature ordinarily employed. The result of the chemical treatment is the production of a fibre which disintegrates easily in the beater after say an hour's beating and gives a sheet of finished paper having high absorptive power for aqueous impregnating compositions, but having no appreciable strength. Rope stock, often mixed with sulphate pulp, is used in the manufacture of saturating papers of the type which are impregnated with glue-glycerine combinations for use as gasket material and the like. Such sheet materials are considerably stronger than the blotting papers, the latter being not adapted for glue-glycerine saturation on account of their low strength. On the other hand gasket materials made from rope fibre have but little absorptive power. This is overcome to some extent by making the paper light and porous by mechanical manipulation on the paper machine, as for example by running the machine very slowly and by eliminating the greater portion of the calendering step on the finished sheet.

According to the present invention a paper product can be made with a high tear resistance and at the same time preserving all the other useful properties of the fibre. This is one of the objects of the invention. Another object is to provide an improved method for cooking vegetable fibres. A further object is to remove fats, wax, and other naturally occurring non-cellulosic materials from raw cotton fibres without

greatly decreasing the strength of the fibres. A still further object is to increase the saturating properties of papers. Yet another object is to prepare saturating papers having an increased strength. It is also an object of the invention to treat such saturating papers with dispersions or solutions of plastic materials such as rubber, glue-glycerine, and other impregnating materials. Other objects will be apparent from the specification and claim.

The invention briefly stated consists in treating cotton fibre with a mild alkaline reagent at a comparatively low temperature for such a period of time that the strength of the fibre is not materially reduced but the waxes, fats, and other naturally occurring materials are removed from the cellulose. The invention also includes forming such cooked fibres into sheets and saturating the sheets thus produced with natural or artificial aqueous dispersions of rubber, with glue-glycerine combinations, with oils and other impregnating compositions known in the arts. The invention contemplates saturating the paper with one or more of the above materials separately or successively or in admixture.

Raw cotton linter or any kind of cotton fibres may be employed as the fibre. Cotton rags or cotton waste may be utilized, but it is preferred to use raw cotton fibre or new rags or waste rather than old material. Waste fibre, such as rags and the like which has previously been cooked to remove the wax, may be mixed with raw cotton fibres, if desired.

In carrying out the invention, 2700 lbs. of raw cotton linter are cooked with 342 lbs. of 58% soda ash (which amounts to about 5-9% on the raw linter) in the presence of 5000 gallons of water. The final concentration of the cooking liquor should not be higher than 0.5%. The cooking can be done in any of the well-known cookers. In this specific illustration a horizontal rotary cooker is used. The cooking is carried out at approximately 230° F. or at a maximum steam pressure of approximately 5 lbs. per sq. inch, the length of time being 1½ hrs. The temperature during the first 40 min. of the cooking does not exceed an average of

120° F. It appears essential that the temperature should not be allowed to become too high. With the steam pressure given above, the time limit for the cooking should not exceed 3 hrs. and it is not desirable to use higher temperatures in order to shorten the cooking time owing to the great increase in the speed of the chemical reaction with comparatively small increase in temperature. The liquor is drained out of the cooker and the latter is filled with clean water and agitated for say 1/2 hr. to wash out the soda. The washing may be carried out just as satisfactorily in a beater washer. 15 An hour's washing in the beater is usually sufficient.

The fibre, cleansed of the fats, wax, etc., is now beaten preparatory to making paper. With the cooking given above and with the 20 type of raw material, 1 1/2 hrs. is usually a sufficient time for the beating. It is pointed out, however, that the beating time may vary with different types of beaters and may be shortened or increased depending on the type 25 of the product desired. The beating is done in conformance with standard practice. The invention is not limited to the proportions given above for these may be varied to meet special requirements without departing 30 from the spirit of the invention.

According to the present invention, it is possible to utilize raw linter which contains 35 husk and hulls. These need not be removed for many purposes, and the retention of these husks and hulls goes hand in hand with the retention of fibre strength, for to remove the husks a prolonged cooking is a required with subsequent loss of strength in the fibres. Filling materials, colors and vulcanizing 40 ingredients (when rubber is incorporated) may be added to the contents of the beater. It may be desirable to use a blend of paper making materials, that is to add wood pulp or other paper stocks together with the 45 cotton fibre.

The saturating paper thus obtained will absorb such materials as glue, glycerine, natural and artificial latex, and other materials in solution or suspension very much 50 more rapidly than the best rope (or mixtures of rope and other fibres) saturating papers. If latex be poured upon a sheet of the paper it will be found that the latex strikes through the paper in a few seconds and appears 55 underneath as latex, indicating that there has been no separation of the rubber from the aqueous portion of the latex. In many instances in the present practice saturation properties may be obtained, but no addition 60 is made to the strength, and frequently there is an actual loss of strength. For example, treating ordinary saturating paper with latex does not add to the strength of the paper. In the present invention, however, 65 treatment with latex materially increases

the strength of the saturating paper. Another illustration of the saturating value of the paper made according to the present invention is the speed with which the paper will absorb the glue-glycerine compositions 70 of the type ordinarily employed in the manufacture of paper gaskets, etc. Ordinary saturating paper will take up 70-80% of its weight of glue-glycerine compound, but the latter must be heated to 140-160° F. in order 75 for proper saturation to take place. With paper made according to the present process, the glue-glycerine mixture need not be heated at all, for at ordinary temperatures it penetrates at least three times as rapidly as the 80 heated composition will penetrate ordinary saturating paper. Latex may be combined with the glue-glycerine composition and the paper saturated at ordinary temperatures. This combination could not be absorbed at 85 all by the usual types of saturating paper for the rubber contained in the mixture would filter out on the surface of the sheet.

With the best grades of saturating papers heretofore known, (after saturation with 90 latex) a tear resistance of 700 by the Elmen-dorf method is well nigh unobtainable, irrespective of whether the paper has been saturated or not. The paper made according to the present invention has a tear resistance of more than 800 on the same weight sheet before saturation and from 800 to 1500 or even higher after treatment with latex or other materials. Tear resistances of this magnitude are unknown in the ordinary manufacture of paper. The present paper saturates much more rapidly and absorbs greater amounts of solution than the ordinary papers. This gives the paper of the present invention a much higher efficiency in the use to which it is put, for it can be made to contain greater amounts of the absorbed material than is possible with the ordinary types of saturating paper. The saturating paper prepared according to the 110 above examples has also the ability to absorb varnishes of various sorts such as the insulating varnishes and other coatings and impregnating liquids used in the various industries. Phenolic condensation products in 115 the liquid stage or in solution may be absorbed into the paper and subsequently hardened. The saturating paper thus prepared lends itself readily to the application of various kinds of coatings in the manufacture of coated papers. Its whole structure permits the ready ingress of adhesive solutions in which respect the paper has a certain utility as a backing for cloth and other surfacing materials.

In the claim, the term "de-waxed" is understood as comprehending the removal of fats, waxes, oils, ligneous matter from the fibres.

Having thus described our invention, what 130

we claim and desire to protect by Letters Patent is:

A process for making sheet material which comprises mildly cooking cotton fibre to remove fats, oils, waxes, and other non-cellulosic material therefrom without impairing the strength of the fibre, making the cooked fibre into a sheet material, and absorbing a

plastic substance from a dispersion thereof into the body of the sheet.

10

Signed at New York, county and State of New York, this 8th day of December, 1925.

REED P. ROSE.

Signed at New York, county and State of New York, this 8th day of December, 1925.

HAROLD E. CUDE.